

# UNITED STATES PATENT OFFICE.

GEORGE M. J. MACKAY, OF SCHENECTADY, NEW YORK, ASSIGNOR TO GENERAL ELECTRIC COMPANY, A CORPORATION OF NEW YORK.

## INCANDESCENT ELECTRIC LAMP.

1,234,060.

Specification of Letters Patent. Patented July 17, 1917.

No Drawing.

Application filed April 30, 1913. Serial No. 764,701.

To all whom it may concern:

Be it known that I, GEORGE M. J. MACKAY, a subject of the King of Great Britain, residing at Schenectady, in the county of 5 Schenectady and State of New York, have invented certain new and useful Improvements in Incandescent Electric Lamps, of which the following is a specification.

My invention relates to incandescent electric lamps and more especially to lamps provided with filaments of high melting point metals such as tungsten. In its preferred embodiment my invention is applied to lamps having filaments of drawn tungsten.

Among the objects of my invention is the production of a lamp in which the efficiency of the lamp shall be maintained fairly constant, and in which the length of life of 10 the lamp shall be greatly increased. This result I accomplish in the particular embodiment hereinafter described, by providing within the lamp bulb a certain small pressure of a gas such as nitrogen, the pressure 15 being so chosen that the tendency of the lamp to decrease in candle power as the filament wastes away and the lamp bulb blackens shall be more or less counteracted by the gradual disappearance of the gas due 20 to the so-called "clean-up" action of the filament thereon. Where the amount of gas in the bulb is suitably proportioned in accordance with my invention, this "clean-up" 25 action gradually removes gas from the space about the filament and thereby the cooling effect of the gas upon the heated filament is decreased. There is thus a tendency for 30 the temperature of the filament to rise, and if the amount of gas has been properly 35 chosen in the first instance, this decreased cooling tendency may be made more or less closely to balance the tendency of the filament to fall in candle power as it slowly wastes away. This gas thus exerts a sort 40 of equalizing effect, for whereas it cools the filament at the beginning of its life, thus necessitating that the filament be run at 45 higher temperature than in vacuum to give the desired efficiency, the cooling automatically becomes less as the lamp continues in 50 operation and fall in candle power and in efficiency is thus lessened or prevented.

Another factor in the reduction of efficiency of an incandescent lamp is the blackening of the bulb due to the deposition

thereon of material evaporated from the filament. In the case of a tungsten filament lamp the color of this deposit is ordinarily black but in a lamp made in accordance with my invention the deposit, where the filament is of tungsten, is distinctly brown, and appears to be tungsten nitrid ( $WN_2$ ), the nitrogen of the compound being derived from the nitrogen gas originally placed in the bulb. The nitrogen does not 60 appear to combine directly with the metal of the filament but with the tungsten which has been driven off from the filament. The deposit of nitrid is lighter in color or tint than is the deposit in the case of a vacuum 65 lamp, and therefore does not cut down so much the transmission of light, and this is a valuable feature in securing increased 70 length of life of the lamp and maintenance of efficiency.

The amount of nitrogen which I find it desirable to place in the bulb of the lamp varies according to the size and length of the filament, though the size of the bulb and the efficiency at which the filament is run 75 80 may slightly modify conditions. The pressure of nitrogen to be used in any particular case with bulbs of the usual size may be roughly estimated as corresponding to about 10 millimeters pressure for every square 85 centimeter of filament surface. With a filament of tungsten 5 mils in diameter and of about 5 inches in length, the best pressure appears to be about 2 millimeters though the beneficial effects of my invention may be 90 obtained with pressures as low as one-tenth of a millimeter up to as high as 5 millimeters. With a filament of say 10 mils in diameter a pressure of about 25 millimeters 95 may to advantage be employed, a higher pressure being allowable with filaments of large diameter on account of relatively less energy loss by conduction through the gas.

It is important that the pressure of nitrogen should not be too low, such, for example 100 as a very small fraction of a millimeter, since in that case the "clean-up" effect is so rapid that the filament is left running at a higher temperature than it is capable of 105 withstanding for a proper length of time, and the bulb discolors very rapidly. On the other hand, if too high a pressure of nitrogen is chosen, then the temperature of the filament, particularly if the filament be of small diameter, must be raised so high in or 110

der to maintain proper efficiency that the lamp soon burns out. In general, the limits of pressure of gas to be employed in the lamp in accordance with my invention may 5 be roughly placed as from one-fifth of a millimeter up to 50 millimeters for each square centimeter of filament surface, depending upon conditions, but the particular pressure to be employed in any particular case should 10 be determined by the considerations which I have mentioned.

Where the pressure of nitrogen in the lamp is properly chosen, I have found that a lamp having a filament of tungsten running 15 in an atmosphere of this pressure has its useful life prolonged to some two or three times that which it would have if the filament were operated in a vacuum, while at the same time the efficiency or watts per candle 20 remains constant within a fair degree of approximation.

My invention is more especially applicable in connection with lamps operating on low voltage since in this case there is less 25 danger due to arcing between the leading-in wires in the lamp.

I am aware that lamps have been constructed in which a small amount of gas probably less than .025 millimeters was purposely 30 allowed to remain in the bulb. After the bulb had been thoroughly evacuated, the filament not having been brought to incandescence during this period, the bulb was sealed off so that thereafter, when the filament was heated to incandescence a certain 35 amount of gas was driven out of the filament. This gas is sometimes known as the "flash gas", consisting probably of carbon monoxide and hydrogen, and this gas remained 40 in the bulb and was observed to have a certain beneficial effect, the nature of which was, however, not understood. In those cases, however the improvement in the life of the lamp was only a few per cent., whereas 45 in lamps made in accordance with my invention an improvement of 200 to 300 per cent. or more has been noted. Moreover, in those lamps to which I refer in which the "flash gas" had been allowed to remain, the 50 appearance of the bulb after operation was

radically different from that of the bulbs of lamps made in accordance with my invention, the deposit on the bulb being of a bluish black color instead of a light brown.

What I claim as new and desire to secure 55 by Letters Patent of the United States, is:

1. In an incandescent electric lamp, the combination of a bulb, a filament therein of tungsten, and a low pressure of gas which is substantially chemically inactive with respect to the filament itself, the pressure being so chosen initially that the progressive "clean-up" of gas during the operation of the lamp produces a progressive decrease in cooling effect on the filament approximately 60 counterbalancing the progressive decrease in heat generated in the filament, due to the wasting away of the filament.

2. An incandescent lamp comprising a bulb, a tungsten filament therein, and a filling of nitrogen therein at an initial pressure corresponding substantially to the proportion of about  $\frac{1}{5}$  of a millimeter up to 50 millimeters of mercury pressure for each square centimeter of filament surface, the 70 pressure progressively decreasing during the operation of the lamp.

3. An electric incandescent lamp comprising a sealed bulb, a tungsten filament therein, and a filling of gas which does not directly attack the filament but which will form a compound with material driven off from the filament, the pressure of the gas being chosen initially to be about 10 millimeters of mercury pressure for every square 80 centimeter of filament surface.

4. An electric incandescent lamp comprising a bulb, a tungsten filament therein about 5 mils in diameter and about 5 inches in length and an initial pressure of nitrogen of 90 about 2 millimeters of mercury, the nitrogen progressively decreasing in pressure with the operation of the lamp.

In witness whereof, I have hereunto set my hand this 28th day of April, 1913.

GEORGE M. J. MACKAY.

Witnesses :

BENJAMIN B. HULL,  
HELEN ORFORD.